# EUROPEAN PATENT SPECIFICATION

(11) **EP 2 147 154 B1**
(45) Date of publication and mention of the grant of the patent: **12.08.2015**
(21) Application number: 08758574.1
(22) Date of filing: 16.05.2008
(51) Int. Cl.: D21H 19/38

(54) **COATING COMPOSITION FOR PAPERS PROVIDING EXCELLENT WATER VAPOR BARRIER PROPERTIES**
BESCHICHTUNGSZUSAMMENSETZUNG FÜR PAPIERE MIT HERVORRAGENDEN WASSERDAMPF-SPERREIGENSCHAFTEN
COMPOSITION DE REVÊTEMENT POUR DES PAPIERS FOURNISSANT D'EXCELLENTES PROPRIÉTÉS DE BARRIÈRE À LA VAPEUR D'EAU

(30) Priority: 18.05.2007 EP 07009924
(43) Date of publication of application: 27.01.2010
(73) Proprietor: Topchim N.V., 2160 Wommelgem (BE)
(72) Inventor: VAN DEN ABBEELE Henk, Jan, Frans, 3294 Diest (BE)
(74) Representative: Laenen, Bart Roger Albert
(86) International application number: PCT/EP2008/003945
(87) International publication number: WO 2008/141771

(56) References cited:
- EP-A- 0 513 452
- WO-A-01/59215
- WO-A-98/51860
- WO-A-98/54410
- WO-A-03/078734
- WO-A-2004/018769
- WO-A-2004/074574
- US-A1- 2004 208 999

## Description

The present invention relates to a composition for surface treatment of paper, paperboard or the like.

There is an ongoing trend to replace paperboard that is laminated with polyethylene films by paperboard that is coated with coatings that do not disturb the recycling process of the paperboard. Polyethylene films have very good water vapour barrier properties, however, the films will not disintegrate during the repulping process upon recycling of the paperboard. From an environmental point of view, there is a need to come up with new products. In an article described by Sridach et all, Paper and Timber Vol .881 No2/2006, a barrier coating has been described based on biodegradable polyesters, so that the coated paperboard will be compostable. However, rather thick layers of the coating are needed to obtain sufficiently good water vapour barrier properties and hence this system is economically not attractive.

Conventional types of barrier coatings applied to paper products include waxes. Although waxes confer excellent barrier properties, they can not be glued or overprinted very easily and are also problematic during the repulping process.

Accordingly, there is need for a water vapour barrier coated cellulosic substrate which is easy and inexpensive to manufacture, has good barrier properties with respect to water and water vapour, can be glued or over-printed easily, and can be easily disposed or recycled.

It is an object of the invention to provide such a coating.

This object is achieved in that the composition on a solid weight basis comprises: 20 to 55% of a binder with a glass transition temperature lower than 30°C; 45 to 80% of a talcum with an average particle size between 50 and 2000nm; and further characterized in that the talcum has an aspect ratio of higher than 30, and a chlorite content between 8 and 30%.

Accordingly to the present invention the composition that provides coatings with good water and water vapour barrier properties are obtained by choosing talcum particles with a specific particle size, combined with a specific weight ratio between the talcum particles and the binder and a specific chlorite content.

For talcum in particular, the mean particle size is generally between 2 and 10 microns and is obtained by dry grinding and selection. However, it is found now that talcum with a smaller particle size has a dramatic effect on the water vapour barrier properties. To obtain these particles with smaller sizes one can use a ball mill delaminating process. The talcum to start with can have an average particle size of a few micrometers or can be more coarse. A way of making these fine talcum particles has been described in patent US 6,348,536. The use of the products described in this patent for paper coatings is part of the present invention. This patent describes a wet grinding process leading to lamella-type minerals in the form of particles constituted of stacks of sheets. The process is characterized by the fact that the mineral is suspended in a liquid with a predetermined initial particle size, after which the suspension is subjected to a delamination procedure in order to separate the sheet from the particles, and obtain a particle size smaller than the initial particle size. Said suspension is then subjected to selection in order to eliminate the particles larger in size than the predetermined size; it is subsequently dried, and the mineral particles are treated so as to restrict the creation amongst them of strong irreversible bonds.

Good results can also be achieved by using a talcum with an average particle size smaller than 2000 nm obtained by a dry or wet milling process. A well-suited apparatus to obtain the requested particles is a Super-Orion Ball mill from Hosokawa Micron. The milling process should in first instance aim at increasing the aspect ratio of the particles. Most of the commercially available talcum products have an aspect ratio of less than 5. Due to ball milling process talcum particles with an average particle size below 2000 nm will start to delaminate, leading to a higher aspect ratio. The use of a talcum with an average particle size smaller than 2000n nm has also been described in WO03078734. Preferably for the present invention the talcum particles have an aspect ratio of more than 30 and more preferably an aspect ratio of more than 50.

It should be noted that talcum with a particle size lower than 500 nm will be too expensive for obtaining water vapour barrier properties but also the hydrophobic properties are less good.

In a preferred embodiment of the invention the specific surface of the talcum is between 10 and 20m²/gr.

Specific for the present invention is that a talcum is used having a chlorite content between 8 and 30%, preferably between 10 and 20%, and more preferably between 10 and 16 %. A talcum that is very suitable for getting optimum water vapour barrier properties is a talcum from the Open mine of Trimouns (Pyrenees-France) that is treated according to the invention described in patent US 6,348,536.

The binder should be very hydrophobic, but should further allow gluing and overprinting of the resultant coating. A good comprise has been found by using styrene butadiene latex as a binder. Other good water borne binders are polyurethane, polyester or polyethyleneacrylate dispersions. The weight ratio between the binder and the talcum particles is chosen so that a maximum weight of talcum particles is obtained in the coating without creating pores in the coating. Dependent on the particle size of the talcum particles the weight ratio between the binder and the talcum particles will be between 20 / 80 and 55 / 45 and more preferably between 33 / 67 and 40 / 60.

The Tg of the binder should preferably be lower than 30°C in order to provide good filming properties during the drying process. A Tg between 10°C and 15°C is most preferred.

For making the coating composition the talcum is dispersed in the water phase. To increase the stability of the dispersion classical dispersion aids can be added. Such a dispersion aid is for example Coatex P. The amount of dispersion aid will preferentially be not higher than 1%. Other additives may be added for instance to limit foaming behavior during the dispersion process.

After dispersing the talcum the water borne binder will be added.

In a preferred embodiment of the invention a weight amount of less than 5% of wax or oil can be added to increase the hydrophobic properties of the coating. Preferably, the amount of wax is less than 2%. Waxes that are suitable are for example parafine wax or fatty acids.

A small amount of a crosslinker such as for instance ammonium zirconium carbonate or formaldehyde resins can be added. Typical amounts of crosslinkers added are less than 3%. Higher amounts may hurt the recyclability of the paper

Low molecular weight organic solvents can be used in combination with water as the liquid carrier and examples thereof include alcohols such as methanol, ethanol, propanol, isopropanol and mixtures thereof. Especially when binders are used with a Tg higher than 30 C solvents are added to improve the film forming properties of the binder.

The coating may contain some other coating additives which are common for paper coating formulations. These can be for example colouring agents, optical brighteners or anti-microbial agents.

In a preferred embodiment of the invention the viscosity of the coating composition is between 10 and 800 centipoises. By doing so a good flow of the coating and an increased penetration of the composition can take place in the pores of the paper product.

The solids content of the formulation should preferably be between 45 and 65%.

In another preferred embodiment of the invention the compositions are applied on the paper or the paperboard by a coating machine having a bend blade, an air knife or a rod. Also curtain coaters are suitable for this application. Applications of the compositions by using machines having a stiff blade clearly showed inferior water vapor barrier properties. Application on paper. Rods to be used.

## Claims

1. Composition for surface treatment of paper, paperboard or the like, **characterized in that** the composition on a solids weight basis comprises:
- 20 to 55% of a binder with glass transition temperature lower than 30°C
- 45 to 80% of a talcum with an average particle size between 500 and 2000 nm; and **in that** the talcum has an aspect ratio of higher than 30, and a chlorite content between 8 and 30 %.

2. Composition according to claim 1 , **characterized in that** the composition on weight basis comprises:
- 33 to 40% of a binder with glass transition temperature lower than 30°C
- 60 to 67% of a talcum with an average size between 500 and 2000 nm.

3. Composition according to claim 1 or 2 **characterised in that** the binder is a styrene butadiene latex.

4. Composition according to any one of the claims 1 - 3 **characterized in that** the talcum has an aspect ratio of higher than 50

5. Composition according to any one of the claims 1 - 4 **characterised in that** the specific surface area of the talcum particles is between 10 and 20m²/gr.

6. Composition according to any one of the claims 1 - 6, **characterized in that** the small particle size of the talcum is obtained by a wet milling process

7. Composition according to any one of the claims 1 - 6, **characterized in that** the solids content is between 45 and 65%.

8. Composition according to any one of the claims 1 - 7, **characterized in that** the viscosity of the formulation is between 10 and 800 centipoise.

9. The application of compositions according to any one of the claims 1 - 8, for making water vapor barrier coatings on paper, paperboard and the like by using a coating machine with a bend-blade, air knife, curtain coater or a rod

10. A cellulosic substrate coated with a composition according to any one of the claims 1 - 9.

## Patentansprüche

1. Eine Zusammensetzung zur Oberflächenbehandlung von Papier, Karton oder ähnlichen Materialien, die **dadurch kennzeichnet ist, dass** sie aus der folgenden Mischung von Inhaltsstoffen besteht (alle Angaben beziehen sich auf das Gewicht):
- zu 20 bis 55 % aus einem Bindemittel mit einer Glasübergangstemperatur von weniger als 30°C,
- zu 45 bis 80 % aus einem Talkum mit einer durchschnittlichen Partikelgröße zwischen 500 und 2000 nm, einem Seitenverhältnis von mehr als 30 und einem Chloritanteil von 8 bis 30 %.

2. Die Zusammensetzung gemäß Anspruch 1, **dadurch kennzeichnet, dass** die Zusammensetzung gewichtsmäßig aus der folgenden Mischung von Inhaltsstoffen besteht:
- zu 33 bis 40 % aus einem Bindemittel mit einer Glasübergangstemperatur von weniger als 30°C,
- zu 60 bis 67 % aus einem Talkum mit einer durchschnittlichen Partikelgröße zwischen 500 und 2000 nm.

3. Die Zusammensetzung gemäß einem der Ansprüche 1 oder 2, **dadurch kennzeichnet, dass** es sich bei dem Bindemittel um Styrol-Butadiene-Latex handelt.

4. Die Zusammensetzung gemäß einem der Ansprüche 1 bis 3, **dadurch kennzeichnet, dass** das Talkum ein Seitenverhältnis von mehr als 50 hat:

5. Die Zusammensetzung gemäß einem der Ansprüche 1 bis 4, **dadurch kennzeichnet, dass** die spezifische Oberflächengröße der Talkumpartikel zwischen 10 und 20m²/gr liegt.

6. Die Zusammensetzung gemäß einem der Ansprüche 1 bis 6, **dadurch kennzeichnet, dass** die geringe Partikelgröße des Talkums durch ein Nassvermahlungsverfahren erreicht worden ist.

7. Die Zusammensetzung gemäß einem der Ansprüche 1 bis 6, **dadurch kennzeichnet, dass** der Feststoffgehalt zwischen 45 und 65 % liegt.

8. Die Zusammensetzung gemäß einem der Ansprüche 1 bis 7, **dadurch kennzeichnet, dass** die Viskosität der Rezeptur zwischen 10 und 800 Centipoise liegt.

9. Die Anwendung von Zusammensetzungen gemäß einem der Ansprüche 1 bis 8 zur Erzeugung von Wasserdampf-Barrierebeschichtungen auf Papier, Karton und ähnlichen Materialien durch Verwendung einer Beschichtungsmaschine mit Bogenklinge, Luftmesser, Curtain Coater oder einem Stab.

10. Ein zellulosisches Substrat, das mit einer Zusammensetzung gemäß einem der Ansprüche 1 bis 9 beschichtet worden ist.

## Revendications

1. Composition pour le traitement de la surface du papier, du carton ou similaire, **caractérisée en ce que** la composition du poids sec des solides comprend :
- 20 à 55% de liant avec une température de transition vitreuse inférieure à 30°C
- 45 à 80% de la une taille de particules moyennes entre 500 et 2000 nm ; et le talc possède un rapport de cadre supérieur à 30, et une teneur en chlorite entre 8 et 30 %.

2. Une composition selon la revendication 1, **caractérisée en ce que** la composition du poids sec comprend :
- 33 à 40% de liant avec une température de transition vitreuse inférieure à 30°C
- 60 à 67% de talc avec une dimension moyenne de 500 à 2000 nm.

3. Une composition selon la revendication 1 ou 2 **caractérisée en ce que** le liant est du latex au styrène butadiène

4. Une composition selon n'importe laquelle des revendications 1-3 **caractérisée en ce que** le talc possède un rapport de cadre supérieur à 50

5. Une composition selon n'importe laquelle des revendications 1-4 **caractérisée en ce que** la surface spécifique de la zone des particules de talc est entre 10 et 20m²/gr.

6. Une composition selon n'importe laquelle des revendications 1-6, **caractérisée en ce que** la petite taille des particules du talc est obtenue par un procédé de mouture humide

7. Une composition selon n'importe laquelle des revendications 1-6, **caractérisée en ce que** la teneur en solides se trouve entre 45 et 65 %.

8. Une composition selon n'importe laquelle des revendications 1-7, **caractérisée en ce que** la viscosité de la formulation se trouve entre 10 et 800 centpoises.

9. L'application des compositions selon n'importe laquelle des revendications 1-8, pour élaborer des revêtements barrières de vapeur d'eau sur le papier, le carton et similaires en utilisant une machine à revêtements avec une lame pliée, une lame d'air, une encolleuse à rideau ou une tige

10. Un substrat cellulosique recouvert d'une composition selon n'importe laquelle des revendications 1 - 9.
